

G. H. HOAGLAND.

Car Axle.

No. 83,159.

Patented Oct 20, 1868.

Fig. 1



Fig. 2



Witnesses:

Adellore  
McKinley

Geo H. Hoagland

# United States Patent Office.

GEORGE H. HOAGLAND, OF PORT JERVIS, NEW YORK.

Letters Patent No. 83,159, dated October 20, 1868; antedated October 10, 1868.

## IMPROVEMENT IN RAILROAD-AXLE.

The Schedule referred to in these Letters Patent and making part of the same.

To all whom it may concern:

Be it known that I, GEORGE H. HOAGLAND, of Port Jervis, in the county of Orange, and State of New York, have invented a new and useful Improvement in Railroad-Axes, of which the following is a full, clear, and exact description, reference being had to the accompanying drawing, forming part of this specification, and in which—

Figure 1 represents a longitudinal view of the end-portion of a railroad-axle, constructed in accordance with my improvement, and

Figure 2 a longitudinal section of the same, with the hub of a wheel arranged thereon.

In locomotive and railroad-car axles, it commonly happens that, while the main body of the axle is sound and unimpaired by usage, the journals are so far worn as to necessitate the replacement of the old axle by a new one, without much or any prospect of utilizing the old one again for the same purpose.

My invention has for its object the remedying of this defect; also, of making new axles more durable than they now are; and consists, in case of manufacturing a new axle, or of repairing an old or worn one, in drawing out or otherwise reducing the ends of the axle, made, as usual, of wrought-iron, and then bringing said ends to a welding or other suitable heat, and casting on or over each of them a steel coat or outer covering, by running the molten metal into a mould, surrounding the end of the axle, to an extent and of a size and shape necessary to form the journal, the steel becoming, by a state of fusion, incorporated with or welded into or on to the drawn or reduced heated end of the wrought-iron axle, after which the axle and journal are hammered into proper shape, and the journal finished as required; and by extending the steel coat thus applied to either end of a wrought-iron axle, beyond the journal, and so as to embrace a portion of the body of the axle, and to enter or be received within, say, one-half the hub of the wheel, thereby giving ample protection to that portion of the axle most liable to break.

Referring to the accompanying drawing, A repre-

sents a wrought-iron railroad-axle, in part, with its end drawn or reduced, as shown in fig. 2. The old or new axle, thus formed, at its opposite ends, has such portions afterwards brought to a red or other suitable heat, successively, as it is preferable to cast the steel coat first on the one end of the axle and then on the other, by placing the axle in a vertical position, and running the molten steel in from above, reversing the ends of the axle uppermost for the purpose. The steel is run into a mould, surrounding the heated end of the axle to give proper size and shape to the coat, which then becomes incorporated with the wrought-iron portion and the whole is afterwards hammered to give proper solidity and shape to axle and journal, and finished as desired.

As represented in the drawing, it is preferred to make the drawn or reduced end *a* longer than the journal *b*, so that the cast-steel coat *B* may be extended to enter wholly or in part the hub *C* of the wheel, say, for half its width, or thereabouts.

A wrought-iron axle, thus provided with steel journals, will of course be much more durable than without the steel wearing-surface, without proportionably adding to the cost of its construction.

I do not claim, broadly, uniting steel with iron, by casting the former on to the latter whilst at a welding heat, and subsequently rolling or swaging the mass into form; nor do I claim a wrought-iron axle, with steel facing, produced in like manner, or by conversion of the exterior in a cementation-furnace, when such steel facing extends the entire length of the axle-shaft; but

What I do claim as new, and desire to secure in Letters Patent, is—

A wrought-iron axle, constructed with steel journal casings, extending about midway into the eye of the wheel, substantially as and for the purposes specified.

GEOR. H. HOAGLAND.

Witnesses:

A. LE CLERC,  
J. W. COOMBS.